

## UNITED STATES PATENT OFFICE.

HATCHIRO FUNASAKA, OF KYOTO, JAPAN.

## PROCESS FOR PERMANENT EMBOSSTMENT OF CLOTH OF ANIMAL FIBER.

No Drawing.

Application filed December 1, 1921. Serial No. 519,099.

*To all whom it may concern:*

Be it known that I, HATCHIRO FUNASAKA, a subject of the Emperor of Japan, residing at No. 13, Shogoin Higashi-machi, Kamikyo-ku, Kyoto, Japan, have invented new and useful Improvements in a Process for Permanent Embosstment of Cloth of Animal Fiber, of which the following is a specification.

10 This invention relates to a process of permanent embosstment of cloth made of animal fiber. Heretofore, cloth was embossed by means of an embossing calender or any such device, but the embossed design on the cloth 15 would disappear in course of subsequent treatment, that is to say, washing or stretching. This difficulty is especially pronounced in cloth made of animal fiber. It may, however, be successfully overcome by my invention.

20 My invented process consists of treating cloth of animal fiber, on which a required design is to be embossed, with a solution of sulphocyanate, and embossing it with a 25 heated calender. To describe further, the cloth is first soaked in a vessel containing a solution of soluble sulphocyanate, for example, sulphocyanate of potash (Baumé 20° to 30°), and, next, the cloth is wrung, then it is 30 pressed by means of a heated embossing calender having engraved thereon the required design. Then the cloth is washed with water, and finally it is dried.

35 By treating cloth with a solution of sulphocyanate, animal fiber is slightly affected and becomes easy to be embossed. When thus treated the cloth is pressed with a 40 heated calender, the fiber of the cloth curls in several grades in accordance with the difference of pressure and that of heating due to the engraving on the surface of the calender, and produces a distinct design on the cloth.

It is preferable that cotton cloth or water-proofed paper or the like, be applied along 45 one, or both sides of the cloth in order to avoid direct contact of the cloth with the calender. This is because the calender is apt to be corroded more or less by the solution of sulphocyanate.

50 In the preceding description, sulphocyanate of potash and an embossing calender are used for the treating agent and the embossing means respectively, but other solutions of soluble sulphocyanate and other 55 pressing means may be alternatively used as the agent and the means respectively to carry out my invention.

What I claim is:—

1. The process of embossing cloth made of 60 animal fiber, which consists in treating the cloth with a solution of sulphocyanate of potash, and then subjecting the cloth under pressure to the action of a heated member having the required design engraved thereon. 65

2. The process of embossing cloth made of animal fiber, which consists in treating the cloth with a solution of sulphocyanate of potash of 20° to 30° Baumé, and then subjecting the cloth under pressure to the action 70 of a heated calender having the required design engraved thereon.

3. The process of embossing cloth made of animal fiber, which consists in treating the cloth with a solution of sulphocyanate of 75 potash, applying to the cloth a protecting layer of material, and subjecting the cloth under pressure to the action of a heated calender having the required design engraved thereon.

80 In testimony whereof I have signed my name to this specification.

HATCHIRO FUNASAKA.